

## UNITED STATES PATENT OFFICE

ERNEST HOPKINSON, OF NEW YORK, N. Y., ASSIGNOR TO THE MECHANICAL RUBBER COMPANY, OF CLEVELAND, OHIO, A CORPORATION OF OHIO

## PAPER PRODUCT AND ITS MANUFACTURE

No Drawing.

Application filed May 27, 1924. Serial No. 716,163.

This invention relates to the manufacture of paper and more particularly to the combination therewith of rubber by a procedure resembling top-sizing.

5 As heretofore practiced, top-sizing has been carried on by passing a web or sheet of paper through a bath of glue or the like and subsequently drying the same. Paper so sized is comparatively stiff, harsh, and only moderately flexible, and its usefulness is limited, being largely confined to ledger and writing papers.

The present invention aims to provide a paper having better strength and durability, 15 a velvety rather than a harsh feel and improved flexibility. The product is suitable not only for writing and ledger papers but also and particularly for map and blue-print papers which are subjected to repeated folding.

With a preferred embodiment in mind but without intention to limit more than is required by the prior art, the invention briefly stated consists in forming a web or sheet of 25 paper pulp and partially drying it before running it through a bath of rubber latex and then completely drying the treated web or sheet.

The web or sheet may be made in any desired 30 way and on any convenient machine, such as those used in the manufacture of paper at the present time. Any suitable paper pulp may be employed and it may or may not have added to it in the beater usual sizing ingredients and/or a small percentage of rubber in a dispersed condition, such for instance as rubber latex diluted to a low rubber content. If natural rubber latex is employed it will 35 preferably contain a small quantity of a preservative such as ammonia or formaldehyde. The web or sheet which has been prepared from paper pulp as above described is then, after being partially dried, passed through a bath of rubber latex whose rubber content 40 may be varied from 4 to 65%. To obtain the required strength of the latex bath, the latex may be either diluted concentrated or thickened in any convenient manner. If the process is carried out on a standard type of paper 45 machine, either a Fourdrinier for paper

sheets or a cylinder machine for thick paper and boards, the web or sheet may be passed down from the drying drums intermediate the length of the battery thereof and into the bath of latex in an incompletely dry condition, then threaded through the second battery of drying drums so that the sizing treatment may be carried on continuously and substantially as heretofore practiced with other sizing solutions. In order to avoid an 55 excess of the rubber latex being carried up from the sizing bath and also to assist in working the latex into the body of the damp web or sheet of partially formed paper, squeeze rolls may be located above the bath 60 or both in and above the bath. The paper may be dried after sizing treatment with latex however festooned in drying lofts or otherwise as convenient instead of on dry cans. After drying the paper may be and is 65 70 preferably calendered.

The properties of the resulting paper will of course depend somewhat upon the properties of the original paper web which is subjected to the top-sizing process with latex. 75 Tests have been carried out on various kinds of paper, viz: sulphite, ground wood, news-print, kraft, manila, rag (ledger), grease-proof, and glassine. In general it has been found that the latex top-sized paper possesses 80 greatly increased folding strength. In some instances papers which have been top-sized with 4-8% rubber latex have over 100% greater folding strength than the same paper without any sizing material. The same is true of the bursting strength of the paper as indicated by a Mullen test. In some cases increase in bursting strength as high as 25% greater than that of the original untreated paper have been obtained where comparatively low amounts of rubber have been retained by the paper. 90

Experiments have been carried out on the various kinds of papers mentioned above, namely, sulphite, ground wood, news-print, 95 kraft, manila, rag (ledger), grease-proof, and glassine, to determine what concentration of rubber latex produces the best results. The concentration varies with the kinds of paper treated, and the purpose for which it is 100

to be used. In general, however, it is noted that so far as increasing the bursting strength of ordinary paper is concerned, there is little to be gained by using a latex which contains more than 8% of rubber solids, although entirely satisfactory results can be obtained with latex of higher concentration. I prefer, however, to use a latex containing between 4-8% of rubber solids. I have also found that in carrying out experiments using the above types of paper web longer immersion in the size bath is required by some than by others, and that the degree the web is dried before immersion in the sizing bath containing latex is widely variable. In some cases the web may approach substantial dryness.

It is to be understood, however, that the invention is not confined to using rubber latex in small proportions as paper may be manufactured with a greater percentage of rubber in the finished paper by either repeatedly passing the same through a dilute latex bath or by using rubber latex which has been thickened or concentrated above its natural strength which lies between 25-35%.

The invention is moreover not confined to the use of rubber latex alone as combinations of the same with vulcanizing ingredients and/or any one or more sizing ingredients, such as water-glass, glue, borated shellac, and casein or other usual sizing ingredients may be employed. These may be mixed in with the rubber-latex or with artificially prepared latex in any manner convenient and in proportions which may be left to the discretion of the manufacturer in order to obtain desired characteristics.

As many apparently widely different embodiments of this invention may be made without departing from the spirit thereof,—in the application of the size containing latex for instance spraying on one or both sides being contemplated as an alternative to passing the web through a bath—it will be understood that I do not intend to limit myself to the specific embodiment herein set forth, except as indicated in the appended claims.

Having thus described my invention, what I claim and desire to protect by Letters Patent is:

1. A process of manufacturing rubberized paper which consists in making a web of paper pulp, removing moisture therefrom, applying thereto a top size containing dispersed rubber, and drying the web to form a sheet.

2. A process of manufacturing rubberized paper which consists in making a web of paper pulp, partially drying the same, top sizing it by continuously passing the web through a sizing bath containing dispersed rubber, and completely drying the web to form a sheet of any desired length.

3. A process of manufacturing rubberized

paper which consists in making a web of paper pulp, partially drying the same, filling in surface irregularities by applying thereto a top size containing rubber latex, and completely drying the web to form a sheet.

4. A process of manufacturing a rubberized paper which consists in continuously forming a web of paper pulp, applying thereto a top size containing rubber-latex of 4-8% solids content, and calendering the treated web to form a finished length of paper.

5. A paper top sized and superficially impregnated with rubber and having a velvety feel, high flexibility, and high resistance to folding, bursting and spreading of inks.

6. A paper product formed by a paper-making process superficially impregnated and surfaced with size containing rubber.

7. A process of manufacturing a rubberized paper which consists in superficially applying size containing rubber latex to a moist sheet of paper pulp while moving, and thereafter drying and calendering the treated sheet to form rubber sized paper.

8. A paper impregnated adjacent its exterior surface only with the dried deposit from rubber latex.

Signed at New York, New York, this 13th day of May, 1924.

ERNEST HOPKINSON.

70

75

80

85

90

95

100

105

110

115

120

125